

Oct. 13, 1942.

L. G. S. BROOKER ET AL

2,298,731

PYRROLE FILTER AND BACKING DYE

Filed Feb. 7, 1940

FIG. 1



FIG. 2



FIG. 3



LESLIE G. S. BROOKER  
ROBERT H. SPRAGUE  
INVENTORS

BY *Paul W. Morris*  
*R. Frank Smith*  
ATTORNEYS

## UNITED STATES PATENT OFFICE

2,298,731

## PYRROLE FILTER AND BACKING DYE

Leslie G. S. Brooker and Robert H. Sprague,  
Rochester, N. Y., assignors to Eastman Kodak  
Company, Rochester, N. Y., a corporation of  
New Jersey

Application February 7, 1940, Serial No. 317,726  
In Great Britain February 17, 1939

5 Claims. (Cl. 95—8)

This invention relates to improvements in photographic elements and more particularly in photographic elements having light screening substances therein.

It is known that photographic elements require, for many purposes, to have light screening substances incorporated therein. Such a light screening substance may be in a layer overlying a light sensitive emulsion or overlying two or more light sensitive emulsions; or it may be in a light sensitive emulsion for the purpose of modifying a light record in such emulsion or of protecting an underlying light sensitive emulsion or emulsions from the action of light of wave length absorbed by such light screening substance; or it may be in a layer not containing a light sensitive substance but arranged between two light sensitive emulsions; or it may be in a layer serving as a backing on an element having one or more light sensitive emulsions (for example, to reduce halation.)

In particular, light screening substances are often required (a) in overcoatings upon photographic elements to protect the light sensitive emulsion or emulsions from the action of light which it is not desired to record, e. g. ultra-violet light in the case of still or moving pictures, especially color pictures, (b) in layers arranged between differentially color-sensitized emulsions, e. g. to protect red- and green-sensitized emulsions from the action of blue light and (c) in backings, forming the so-called anti-halation layers, on either side of a transparent support carrying the light-sensitive emulsion or emulsions.

In most cases, and especially when the element contains a color-sensitized emulsion or color-sensitized emulsions, it is particularly desirable to employ light-screening substances which do not affect the general sensitivity or the color sensitivity of light-sensitive emulsions with which they may come into contact. It is also particularly desirable to employ light-screening substances which do not substantially diffuse from the layers or coatings in which they are incorporated, either during the manufacture of the element or on keeping it or in photographically processing it. Finally, it is generally necessary to employ light-screening substances which can readily be rendered ineffective, i. e. decolorised

or destroyed and removed, prior to or during or after photographic processing; for many purposes it is particularly convenient to employ light-screening substances which are rendered ineffective by one of the photographic baths employed in processing the element after exposure, e. g. a photographic developing bath or fixing bath or a silver-oxidizing (including silver-removing) bath. For example, in an element which is to be processed by reversal, it is often convenient to employ a light screening substance which is rendered ineffective by the developer employed to develop the latent image or images to silver since exposure to light of the residual light sensitive emulsion or emulsions may thereby be facilitated. This is particularly the case when, in making color photographs, several differentially color-sensitized emulsions, constituted, for example, by silver halide, such as silver bromide dispersed in gelatin, collodion or other colloid, are coated on one or both sides of a support, for example in inseparably-superimposed layers. Such differentially color-sensitized emulsions have to be processed to different colors and to facilitate the differential color-processing, methods involving selective exposure of light sensitive images in the layers may be employed. Such selective re-exposure, e. g. of silver halide remaining undeveloped in development of the latent images formed in silver halide emulsion layers (residual silver halide) is often facilitated if the light-screening substance which was present during the original exposure is decolorized or removed in the developing bath employed to develop the latent images to silver. Any of the elements referred to above may be such that one or more of the emulsions contain coupling components, e. g. those described in French Patent 834,371, granted August 16, 1938.

40 Numerous substances have been employed as light-screening substances for the purposes indicated above. Many of these are known yellow dyes but it is has proved extremely difficult to find dyes having the combination of qualities desired. 45 Many are not resistant to diffusion and wander rather freely from the layer in which it is intended that they should remain; many adversely affect the sensitivity of light sensitive emulsions with which they come into contact (a number of 50 these reduce the general sensitivity or some

specific color sensitivity thereof, but others of them may even impart an additional and unwanted specific color sensitivity thereto.

We have now found a class of dyes, members of which fulfill to a very satisfactory extent the requirements of light-screening substances for use in photographic elements. This class consists of polymethine dyes derived from pyrrole or indole or from their substituted derivatives.

Such dyes may have a pyrrole nucleus or an indole nucleus (in either case containing substituents or not) linked to a heterocyclic nucleus containing a nitrogen atom either directly or through an intermediate polymethine chain so that in either case there is a chain, comprising an odd number of carbon atoms having conjugated double linkages between the nitrogen atoms.

In the drawing, the figures are enlarged sectional views of photographic elements showing overcoating, filter, and halation layers according to our invention.

The compounds which we propose to use as screening dyes have the following general formula:



where

Z=the non-metallic atoms necessary to complete a heterocyclic nucleus

J=the non-metallic atoms necessary to complete a pyrrole nucleus

R=hydrogen, alkyl or a chemical bond of a pyridine ring

R'=alkyl

R''=hydrogen, alkyl, aryl or a chemical bond of the same pyridine ring as R

d=2 or 3

n=1 or 2

X=an acid radical

The general formula indicates that the compounds may be depicted in two electomeric forms.

#### Example 1



2.2 g. (1 mol.) 2-β-acetanilidovinylbenzoxazole ethiodide, 2.4 g. (1 mol.+500%) N-methylpyrrole and 10 cc. acetic anhydride were boiled 7 minutes with stirring in a test tube. Dye separated from the boiling mixture. Chilled, filtered, washed with acetic anhydride and acetone and dried. Yield 1.7 g. The product appeared to be a mixture of unchanged starting material and the desired dye. The dye was obtained fairly pure by chilling the solution of the crude product in 50 cc. abs. EtOH for 30 minutes, whereupon the dye separated as red crystals. The mixture was filtered as soon as yellow crystals started to separate. Yield .5 g., 26%. M. P. 264-266° with

decomposition. After a further recrystallization from abs. EtOH, (100 cc./g.) the product was obtained as red crystals melting with decomposition at 265-267°.

#### Example 2



4.34 g. (1 mol.) 2-β-acetanilidovinylbenzoxazole ethiodide, 5.26 g. (1 mol.+100%) 1-lauryl-2,5-dimethylpyrrole and 20 cc. of acetic anhydride were refluxed 10 minutes. The orange reaction mixture was chilled, product filtered off, washed with acetone and water and dried. Yield 4.4 g., 78%. After recrystallization from abs. EtOH, (10 cc./g.) the product was obtained as orange crystals melting with decomposition at 206-207°. Yield 3.7 g., 66%.

*1-lauryl-2,5-dimethylpyrrole*.—Prepared by the method of Lions et al. Proc. Royal Soc. New South Wales, 1937, 71, 92 from laurylamine. B. P. 152-155°/2 mm. Yield 75%.

*1-lauryl-2,5-dimethyl-3-pyrrole aldehyde*.—52.6 g. (1 mol.) 1-lauryl-2,5-dimethylpyrrole, 36 g. (1 mol.+300%) formamide, 35 g. (1 mol.+100%)  $\text{PCl}_3$  and 200 cc. absolute ether was allowed to stand at room temperature for 24 hrs. The yellow solid which separated was filtered off, washed with abs. ether and dried. The solid was suspended in water, made alkaline with stirring and cooling, and the product filtered off, washed with water and dried in vacuum desiccator over  $\text{CaCl}_2$ . Crude yield 40.0 g., 69%. After recrystallization from pet. ether the product was obtained as nearly colorless crystals melting at 60-61°.

#### Example 3



(3-ethyl-2-benzothiazole)-(1-lauryl-2,5-dimethyl-3-pyrrole)-dimethinecyanine-p-toluenesulfonate

1.75 g. (1 mol.) 2-methylbenzothiazole-etho-p-toluenesulfonate, 1.46 g. (1 mol.) 1-lauryl-2,5-dimethyl-3-pyrrole aldehyde and 10 cc. of acetic anhydride were refluxed 5 minutes. The orange reaction mixture was chilled, diluted with 50 cc. of ether and the product filtered off. The red crystals were washed with acetone and water and dried. Yield 1.5 g., 48%. After recrystallization from abs. EtOH, (28 cc./g.) the product was obtained as vermillion crystals melting with decomposition at 181-182°.

#### Example 4



(1-methyl-2-quinoline)-(1-lauryl-2,5-dimethyl-3-pyrrole)-dimethinecyanine-p-toluenesulfonate

3.3 g. (1 mol.) quinaldine metho-p-toluenesulfonate, 2.9 g. (1 mol.) 1-lauryl-2,5-dimethyl-3-pyrrole aldehyde, 5 drops of piperidine and 15 cc. of absolute EtOH were refluxed 10 minutes. The orange solution was cooled, diluted to 300 cc. with 5 ether and chilled. The dye was filtered off, washed with water and acetone and dried. Yield 5.2 g., 87%. After recrystallization from abs. EtOH, (12 cc./g.) the product was obtained as red crystals melting with decomposition at 10 163-165°. Yield 3.4 g., 57%.

*Example 5*



3-[(3-ethyl-2(3-benzoxazolylidene) ethylidene]-2-methyl-indolenine hydro-iodide

2.2 g. (1 mol.) 2- $\beta$ -acetanilidovinylbenzoxazole ethiodide, 2.6 g. (1 mol.+100%)  $\alpha$ -methylindole and 10 cc. of acetic anhydride were boiled 3 minutes in a test tube. Dye separated from the boiling solution. Chilled, filtered, washed with water and acetone and dried. Yield 1.4 g., 65%. After recrystallization from MeOH, (120 cc./g.) the product was obtained as brown needles with metallic reflex melting with decomposition at 287-288°. Yield 1.25 g., 58%.

*Example 6*



3-[(3-ethyl-2(3-benzothiazolylidene) ethylidene]-2-methyl-indolenine hydro-iodide

2.25 g. (1 mol.) 2- $\beta$ -acetanilidovinylbenzothiazole ethiodide, 2.6 g. (1 mol.+100%)  $\alpha$ -methylindole and 15 cc. of acetic anhydride were refluxed 5 minutes. The orange solution was chilled, filtered, the dye washed with acetone and water and dried. Yield 1.8 g., 81%. After recrystallization from MeOH, (200 cc./g.) the product was obtained as minute red crystals with metallic reflex melting with decomposition at 290-292°.

*Example 7*



(3-ethyl-2-benzoxazole)-(1-ethyl-3-indole)-di-methinecyanine iodide

2.2 g. (1 mol.) 2- $\beta$ -acetanilidovinylbenzoxazole ethiodide, 1.5 g. (1 mol.+100%) 1-ethylindole and 10 cc. acetic anhydride were boiled in a test tube for 5 minutes. The orange solution was chilled, filtered, the dye washed with acetone and water and dried. The product appeared to be a mixture of the desired dye with unchanged starting material. Wt. 1.8 g. This was extracted with EtOH and the dye isolated from the more soluble fraction as orange-red crystals. Yield 3 g., 14%. After recrystallization from abs. EtOH the dye melted at 247-249° with decomposition. Yield 25 g., 11%.

5  
10

3-[(3-ethyl-2(3-benzoxazolylidene) ethylidene]-2-hexylindolenine hydro-iodide

20

4.34 g. (1 mol.) 2- $\beta$ -acetanilidovinylbenzoxazole ethiodide, 2.7 g. (1 mol.+35%) 2-hexylindole and 15 cc. of acetic anhydride were refluxed 5 minutes. Dye separated from the boiling solution. Chilled, filtered, washed with acetone and water and dried. Yield 2.8 g., 56%. After recrystallization from MeOH the product was obtained as minute brown crystals with metallic reflex melting with decomposition at 272-274°. Yield 1.4 g., 28%.

25



(3-ethyl-2-benzoxazole)-(1,2-dimethyl-3-indole) dimethinecyanine iodide

30

.87 g. (1 mol.) 1,2-dimethyl-3-indolealdehyde, 1.45 g. (1 mol.) 2-methylbenzoxazole ethiodide and 10 cc. acetic anhydride were refluxed 5 minutes. Orange coloration. Solid dye separated from the boiling reaction mixture. Chilled, filtered, washed with water and acetone and dried. Yield of brownish yellow crystals 2.15 g., 97%. After recrystallization from MeOH (50 cc./g.), the product was obtained as orange crystals melting with decomposition at 264-265°. Yield 2.0 g., 90%. MeOH solution yellow.

35

*Example 9*



(3-ethyl-2-benzoxazole)-(2,5-dimethyl-1-phenyl-3-pyrrole) dimethinecyanine iodide

40

4.35 g. (1 mol.) 2- $\beta$ -acetanilidovinylbenzoxazole ethiodide, 6.0 g. (1 mol.+300%) 2,5-dimethyl-1-phenylpyrrole and 25 cc. acetic anhydride were refluxed 15 minutes. The orange mixture was chilled, filtered, product washed with water and acetone and dried. Brown crystals. Yield 2.7 g., 57%. After recrystallization from MeOH, (15 cc./g.) the dye was obtained as light brown crystals melting with decomposition at 214-220°. Yield 1.6 g., 34%. After three further crystallizations from abs. EtOH with Norite the M. P. was constant at 249-251° dec. MeOH solution yellow.

45

50

*Example 11*



(1-benzyl-2,5-dimethyl-3-pyrrole)-(3-ethyl-2-benzoxazole) dimethinecyanine iodide

55

60

65

70

75

4.34 g. (1 mol.) 2- $\beta$ -acetanilidovinylbenzoxazole ethiodide, 3.7 g. (1 mol. + 100%) 1-benzyl-2,5-dimethylpyrrole and 15 cc. acetic anhydride were refluxed for 10 minutes. Brownish orange coloration. Chilled, filtered, washed with acetone and water and dried. Yield of brown crystals 3.1 g., 64%. After recrystallization from abs. EtOH, (20 cc./g.) the product was obtained as granular brown crystals melting with decomposition at 219-221°. Yield 2.0 g., 41%. MeOH solution yellow. 10

## Example 12



(3-ethyl-2-benzoxazole)-(1-p-methoxy-phenyl-2,5-dimethyl-3-pyrrole) dimethinecyanine iodide

4.34 g. (1 mol.) 2- $\beta$ -acetanilidovinylbenzoxazole ethiodide, 4.0 g. (1 mol. + 100%) 2,5-dimethyl-1-p-methoxy-phenylpyrrole and 15 cc. acetic anhydride were refluxed 15 minutes. Orange coloration. Chilled, filtered, washed with acetone and water and dried. Brown crystals. Yield 2.5 g., 50%. After recrystallization from abs. EtOH, (11 cc./g.) the product was obtained as granular brown crystals melting with decomposition at 214-217°. Yield 1.9 g., 38%. MeOH solution yellow. 35

## Example 13



(1-octadecyl) (1-cetyl) (2,5-dimethyl-3-pyrrole)-(3-ethyl-2-benzoxazole) dimethinecyanine iodide

4.34 g. (1 mol.) 2- $\beta$ -acetanilidovinylbenzoxazole ethiodide, 6.4 g. (1 mol. + 100%) mixture of 1-cetyl-2,5-dimethylpyrrole and 1-octadecyl-2,5-dimethylpyrrole and 20 cc. acetic anhydride were refluxed 5 minutes. Chilled, filtered, washed with acetone and water and dried. Brown crystals. Yield 4.1 g., 66%. After recrystallization from abs. EtOH (5 cc./g.) the product was obtained as brown needles melting with decomposition at 180-183°. Yield 3.7 g., 60%. MeOH solution yellow. 55

## Example 14



(1-p-dimethylaminophenyl-2,5-dimethyl-3-pyrrole)-3-ethyl-2-benzoxazole dimethinecyanine iodide

4.34 g. (1 mol.) 2- $\beta$ -acetanilidovinylbenzoxazole ethiodide, 4.3 g. (1 mol. + 100%) 1-p-dimethylaminophenyl-2,5-dimethyl-pyrrole and 75

15 cc. acetic anhydride were refluxed 10 minutes. Orange coloration. Chilled, filtered, washed with acetone and water and dried. Yield 4.3 g., 84%. After recrystallization from MeOH, (33 cc./g.) the product was obtained as brown crystals with a bright reflex melting with decomposition at 264-266°. Yield 3.75 g., 74%. MeOH solution yellow.

## Example 15



(3- $\beta$ -hydroxyethyl-2-benzothiazole)-(1-lauryl-2,5-dimethyl-3-pyrrole) dimethinecyanine bromide

2.9 g. (1 mol.) 1-lauryl-2,5-dimethyl-3-pyrrole-aldehyde, 2.74 g. (1 mol.) 2-methyl-benzothiazole- $\beta$ -hydroxyethobromide, 5 drops piperidine and 15 cc. abs. EtOH were refluxed 10 minutes. Orange coloration. Chilled, filtered, washed with acetone and water and dried. Yield of yellow crystals 4.05 g., 73%. After recrystallization from abs. EtOH, (10 cc./g.) the product was obtained as brownish orange crystals melting with decomposition at 234-235°. Yield 3.6 g., 66%. MeOH solution yellow. 20 25 30 35

## Example 16



(3-ethyl-2-benzoxazole)-(2-phenyl-1-pyrrocoline) dimethinecyanine iodide

1.93 g. (1 mol.) 2-phenylpyrrocoline, 4.34 g. (1 mol.) 2- $\beta$ -acetanilidovinyl-benzoxazole ethiodide and 25 cc. glacial acetic acid were refluxed 10 minutes. Red coloration. Chilled, filtered, washed with acetone and water and dried. Yield of red crystals 4.45 g., 91%. After recrystallization from abs. EtOH, (19 cc./g.) the product was obtained as granular red crystals melting with decomposition at 204-205°. Yield 3.9 g., 79%. MeOH solution orange. 50

## Example 17



(3-ethyl-2-benzoxazole)-(2-methyl-1-pyrrocoline) dimethinecyanine iodide

4.34 g. (1 mol.) 2- $\beta$ -acetanilidovinylbenzoxazole ethiodide, 1.3 g. (1 mol.) 2-methylpyrrocoline and 15 cc. glacial acetic acid were refluxed 5 minutes. Red coloration. Chilled, filtered, washed with acetone and water and dried. Yield of green crystals 3.85 g., 90%. After recrystallization from MeOH, (39 cc./g.) the dye was obtained as green crystals with a golden reflex melting with decomposition at 245-246°. Yield 3.2 g., 75%. MeOH solution orange. 60 65 70 75

## Example 18



(3-ethyl-2-benzoxazole)-(1-β-methoxyethyl-2,5-dimethyl-3-pyrrole) dimethinecyanine iodide

4.34 g. (1 mol.) 2-β-acetanilidovinylbenzoxazole ethiodide, 3.0 g. (1 mol. + 100%) 1-β-methoxyethyl-2,5-dimethylpyrrole and 15 cc. acetic anhydride were refluxed 10 minutes. The brownish-yellow mixture was chilled, 100 cc. ether added and again chilled with stirring. The dye which separated was filtered off, washed with acetone and water and dried. Yield of brown crystals 3.5 g., 77%. After recrystallization from abs. EtOH, (14 cc./g.) the dye was obtained as brown crystals melting with decomposition at 219-221°. Yield 2.7 g., 60%. MeOH solution yellow.

## Example 19



(3-ethyl-2-benzoxazole)-(2,5-dimethyl-1-tetrahydrofuryl-3-pyrrole) dimethinecyanine iodide

4.34 g. (1 mol.) 2-β-acetanilidovinylbenzoxazole ethiodide, 3.6 g. (1 mol. + 100%) 2,5-dimethyl-1-tetrahydro furfurylpyrrole and 25 cc. acetic anhydride were refluxed 10 minutes. Brownish orange coloration. Chilled, filtered, washed with acetone and water and dried. Yield 3.8 g., 79%. After recrystallization from MeOH, (24 cc./g.) the dye was obtained as brown crystals melting with decomposition at 250-251°. Yield 3.35 g., 70%. MeOH solution yellow.

## Example 20



(3-ethyl-2-benzoxazole)-(1-cyclohexyl-2,5-dimethyl-3-pyrrole) dimethinecyanine iodide

4.34 g. (1 mol.) 2-β-acetanilidovinylbenzoxazole ethiodide, 3.54 g. (1 mol. + 100%) 1-cyclohexyl-2,5-dimethylpyrrole and 25 cc. acetic anhydride were refluxed 10 minutes. Orange coloration. Chilled, dye ppt'd with 100 cc. ether, ether decanted off and residue stirred with 10 cc. acetone until crystalline. Filtered, washed with acetone and water and dried. Yield 2.25 g., 45%. After recrystallization from abs. EtOH, (13 cc./g.) the dye was obtained as orange needles melting with decomposition at 250-252°. Yield 2.0 g., 42%. MeOH solution yellow.

## Example 21



(3-carbethoxy-2,5-dimethyl-4-pyrrole)-(3-ethyl-2-benzoxazole) dimethinecyanine iodide

5.8 g. (1 mol.) 2-methylbenzoxazole ethiodide, 3.9 g. (1 mol.) 3-carbethoxy-2,5-dimethyl-4-pyrrolealdehyde, 5 drops piperidine and 30 cc. n-propylalcohol were refluxed 20 minutes. Orange coloration. Chilled, filtered, washed with acetone and water and dried. Yield of yellow crystals 2.55 g., 27%. After recrystallization from abs. EtOH, (12 cc./g.) the dye was obtained as yellow crystals melting with decomposition at 226-227°. Yield 1.7 g., 18%. MeOH solution yellow.

25

## Example 22



(3-ethyl-2-benzoxazole)-(2,3-dimethyl-1-pyrrocoline) dimethinecyanine iodide

35

4.34 g. (1 mol.) 2-β-acetanilidovinylbenzoxazole ethiodide, 1.5 g. (1 mol.) 2,3-dimethylpyrrocoline and 25 cc. glacial acetic acid were refluxed 5 and 25 minutes. Red coloration. Chilled, stirred until crystalline, again chilled and filtered. Washed with acetone and water and dried. Yield of dark red crystals 3.85 g., 87%. After recrystallization from MeOH, (42 cc./g.) the dye was obtained as greenish-red needles with green-reflex melting with decomposition at 266-267°. Yield 3.55 g., 80%. MeOH solution orange.

50

## Example 23



(1-lauryl-2,5-dimethyl-3-pyrrole)-(1,3,3-trimethyl-2-indole) dimethinecyanine iodide

60

3.0 g. (1 mol.) 2,3,3-trimethylindolenine methiodide, 2.9 g. (1 mol.) 1-lauryl-2,5-dimethyl-3-pyrrolealdehyde, 5 drops piperidine and 15 cc. abs. EtOH were refluxed 1 hour. Orange coloration. Cooled, 3.0 g. (1 mol. + 100%) NaI in 15 cc. MeOH added and mixture diluted to 150 cc. with ether. Orange-red crystals separated. Chilled, filtered, washed with ether and water and dried. Yield 3.1 g., 54%. After recrystallization from abs. EtOH, (8 cc./g.) the dye was obtained as bright red flakes melting with decomposition at 283-285°. Yield 2.0 g., 35%. MeOH solution orange.

75

## Example 24



3-[4-(3-ethyl-2(3)-benzothiazolylidene)-2-butenyldene]-2-methylindolenine hydrobromide

2.6 grams (1 mol.) 2-(4-acetanilido-1,3-buta-  
dienyl)-benzothiazole ethiodide, 1.3 grams (1  
mol. +100%)  $\alpha$ -methylindole and 15 cc. acetic  
anhydride were refluxed 10 minutes. The purple  
reaction mixture was chilled, the dye which sepa-  
rated filtered off and washed with water and  
acetone. The green crystals of dye were dis-  
solved in 150 cc. of hot  $\text{CH}_3\text{OH}$ , filtered and solu-  
tion of excess NaBr in water added. Chilled,  
product filtered off, washed with acetone and  
water and dried. Blue crystalline product. Yield  
.65 gram, 31% after recrystallization from  
 $\text{CH}_3\text{OH}$ , (100 cc./g.) the dye was obtained as  
blue crystals melting with decomposition at 269-  
270°. Yield .4 gram, 19%.  $\text{CH}_3\text{OH}$  solution red.

## Example 25



(3-ethyl-2-benzothiazole)-(2-phenyl-1-pyrrocoline) tetramethine cyanine chloride

4.8 grams (1 mol.) 2-(4-acetanilido-1,3-buta-  
dienyl)-benzothiazole ethiodide, 1.93 grams (1  
mol.) 2-phenyl-pyrrocoline and 30 cc. glacial  
acetic acid were refluxed 3 minutes. Blue color-  
ation and green crystals of dye separated at once  
from the boiling mixture. Chilled, filtered,  
washed with acetone and water and dried. Yield  
2.6 grams, 49%. The product was extracted with  
700 cc. boiling  $\text{CH}_3\text{OH}$ . Residue of green crystals  
1.3 grams, M. P. 257-259°. The solution was  
chilled and yielded .65 gram green needles, M. P.  
257-259° side by side with above. Combined  
yield 37%. The dye was converted to chloride in  
50 cc. cresol solution using 100% excess freshly  
precipitated silver chloride. The mixture was  
stirred mechanically for 15 hours at 100°, filtered  
hot and chilled. Diluted to 400 cc. with ether  
and chilled overnight. The green crystals which  
separated were filtered off, washed with ether and  
acetone and dried. Yield 1.6 grams, 36%. After  
recrystallization from absolute EtOH, (15 cc./g.)  
the product was obtained as green needles with  
bronze reflex melting at 85-86°, yield 1.3 grams,  
30%.  $\text{CH}_3\text{OH}$  solution bluish-red.

## Example 26



(3-ethyl-2-benzoxazole)-(2-methyl-1-pyrrocoline)-tetramethine cyanine iodide

4.6 grams (1 mol.) 2-(4-acetanilido-1,3-buta-  
dienyl)-benzoxazole ethiodide, 1.3 grams (1 mol.)  
2-methyl-pyrrocoline and 30 cc. glacial acetic acid

10

were refluxed 5 minutes. Blue coloration. Green  
crystals separated at once from the boiling mix-  
ture. Yield 2.9 grams, 64%. Dissolved in 50 cc.  
cresol (m and p mixture) heated to 125°, filter-  
ed hot, cooled and diluted with 250 cc.  $\text{CH}_3\text{OH}$ .  
Green crystals separated on chilling. Filtered,  
washed with  $\text{CH}_3\text{OH}$  and dried. Yield 1.95 grams,  
43%, M. P. 247-250° dec.  $\text{CH}_3\text{OH}$  solution blue.

## Example 27



(3-ethyl-2-benzothiazole)-(2,3-dimethyl-1-pyrrocoline)-  
tetramethine cyanine p-toluenesulfonate

20 4.9 grams (1 mol.) 2-(4-acetanilido-1,3-buta-  
dienyl)-benzothiazole - etho-p-toluenesulfonate,  
1.45 grams (1 mol.) 2,3-dimethylpyrrocoline and  
25 cc. glacial acetic acid were refluxed 5'. The  
blue solution was cooled, diluted with 50 cc. ace-  
tone and 100 cc. ether and chilled. The dye which  
separated was filtered off, washed with ether,  
acetone and water and dried. Yield of green  
crystals, 2.3 grams, 43%. After recrystallization  
from MeOH (32 cc./g.) the product was obtained  
as bright green crystals melting with decomposi-  
tion at 272-273°. Yield 2.0 g., 38%. Solution  
blue in MeOH.

25 In the present specification we refer to dyes  
containing a "pyrrole nucleus." It is to be un-  
derstood that by this term we intend to include  
dyes derived from both pyrrole and indole, the  
indole nucleus being considered a substituted  
pyrrole, and the term "pyrrole nucleus" being  
generic to both pyrrole and indole. While we  
refer in the claims to dyes containing a pyrrole  
nucleus, we intend to include both pyrrole and  
indole dyes.

30 For the preparation of overcoating layers, filter  
layers and anti-halation layers, according to our  
invention, from 50 mg. to 150 mg. of dye are dis-  
solved in from 2 to 5 cc. of a water-miscible  
45 solvent. Methanol or acetone are suitable for  
this purpose but pyridine or Cellosolve may also  
be used. The solution is then added to about 25  
50 cc. of a 5% gelatin solution at 40° C. and the  
mixture coated on the support. If the dye is too  
55 insoluble as the iodide salt it may conveniently  
be converted into the chloride, using cresol as a  
solvent for the conversion.

60 In the accompanying drawing, the various  
figures are enlarged section views of photo-  
graphic elements having filter layers and anti-  
halation layers made according to our invention.  
As shown in Fig. 1 a support 10 of any suitable  
material such as cellulose nitrate or cellulose  
acetate, synthetic resinous material, or opaque  
65 material such as paper is coated with an emulsion  
layer 11 and an overcoating layer 12 containing  
a pyrrole polymethine dye according to our  
invention.

70 Fig. 2 illustrates a multi-layer photographic  
element for color photography in which the sup-  
port 10 is coated with sensitive layers 13, 14  
and 15 which record respectively the red, green  
and blue regions of the spectrum. Between the  
emulsion layers 13 and 14, there is a filter layer  
16 containing a red pyrrole polymethine dye and  
75 between the layers 14 and 15 there is a layer 17  
containing a yellow pyrrole polymethine dye.

These filter layers serve purposes well known in color photography of preventing exposure of a lower layer of the element by light which the filter layers absorb. The pyrrole polymethine dyes used may also absorb light in other regions, such as ultra-violet light.

Fig. 3 represents a film having an anti-halation layer containing a pyrrole polymethine dye according to our invention. As shown therein, the support 10 contains an emulsion layer 11 on one side and an anti-halation layer 18 containing the pyrrole dye on the opposite side.

Our invention is not limited to the examples included in the present specification but any compounds coming within the scope of the invention may be used. The dyes may be dispersed in gelatin, collodion, gum arabic, synthetic resins or other suitable colloid or they may be dispersed in photographic emulsions such as gelatino silver halide emulsions and may be coated in any suitable manner.

It is to be understood that our invention is limited only by the scope of the appended claims.

We claim:

1. A photographic element comprising a sensitive layer and a light absorbing layer containing a dye having the following formula:



in which Z=the non-metallic atoms necessary to complete a heterocyclic nucleus; J=the non-metallic atoms necessary to complete a pyrrole nucleus; R=hydrogen, alkyl, or a chemical bond of a pyridine ring; R'=alkyl; R''=hydrogen, alkyl, aryl, or a chemical bond of the same pyridine ring as R; d=a positive integer of from 2 to 3; n=a positive integer of from 1 to 2; and X=an acid radical.

2. A sensitive photographic element comprising a filter layer containing a dye having the general formula expressed in claim 1.

3. A sensitive photographic element comprising a filter layer containing a (3-alkyl-2-benzoxazole)-(3-pyrrole)dimethinecyanine salt.

4. A sensitive photographic element comprising a filter layer containing a (3-alkyl-2-benzothiazole)-(3-pyrrole)dimethinecyanine salt.

5. A sensitive photographic element comprising a filter layer containing a (3-alkyl-2-benzoxazole)-(1-lauryl-2,5-dimethyl-3-pyrrole)dimethinecyanine salt.

LESLIE G. S. BROOKER.  
ROBERT H. SPRAGUE.